

## UNITED STATES PATENT OFFICE

2,473,190

METHOD OF PRODUCING FIBROUS  
BUILDING COMPOSITIONS

Charles M. Baskin, Toronto, Ontario, and Norman W. McLeod, Sarnia, Ontario, Canada, assignors to Standard Oil Development Company, a corporation of Delaware

No Drawing. Application July 1, 1944, Serial No. 543,196. In Canada July 19, 1943

13 Claims. (Cl. 92—21)

1

This invention relates to improvements in the methods of manufacturing paper, paper felt, and paper boards, and particularly in the manufacture of paper, paper felt, and paper boards that are impervious to moisture and water, and capable of high resistance to damage under handling and other stresses, even when subjected to extreme temperature changes.

Fibrous pulp is produced principally by mechanical grinding whereby the wood or other pulp-forming material such as bagasse from waste sugar cane, salt hay, etc. is disintegrated or pulverized by rough stones rotating against the grain, by hammer mills or other disintegrators and by chemical digestion. In either case, the pulp before it is processed and converted into paper, cardboard or building board, is always diluted with water. Pulp as produced is really a suspension of small quantities of fibre in large quantities of water. In the process of producing roofing paper, the pulp is first made into a paper, or as it is commonly known in the roofing industry, felt. This felt is then transported to the roofing plant and treated by saturating with flux oil, asphalt, or a mixture of flux oil and asphalt, then coated with a higher melting point asphalt, which coating is imbedded with various types of mineral covering material and the sheet is then made up in rolls or cut into shingles. In the production of roofing, the paper sheet or felt, contains as a rule, very little mechanical wood pulp but is largely disintegrated and pulped rags, and some chemically digested long-fibre wood pulp.

Another object of this invention is to provide a method whereby bitumen impregnated paper, paper felt, or paper boards, are turned out directly from a paper making, or paper board making machine, and the necessity for the present process of saturating with a bituminous material is eliminated.

Another object of this invention is to provide a method for turning out waterproof or moisture proof paper, paper felt, or paper boards, directly from a paper making or paper board making machine, in which the bituminous material is contained in the inner portion of the paper sheet, paper felt, or paper board, but does not show on the outside layers. This is an improvement over existing methods, and eliminates the necessity for the present process of laminating two or more sheets of paper using bituminous cements.

A further object of this invention is to modify the characteristics of the waterproofed paper, paper felt, or paper board, by incorporating heavy metal salts of organic acids, such as aluminum naphthenate, copper naphthenate, etc., into the

2

bituminous materials used for waterproofing and cementing.

Other objects of this invention will be more readily understood after reading the following description.

According to this invention, bagasse or other fibrous material was broken up or pulverized in a hammer mill and mixed with flux oil up to an amount of about  $\frac{1}{2}$  part of flux oil to 1 part of fibre. This mixture was then charged into a stationary pressure cooker and digested with a 1.5° Bé. solution of caustic soda at 100 lbs. pressure for 2 hours. The digested mass was beaten and reduced to a fairly fine pulp, during which process the pulverized asphalt and additional flux oil was added to give an overall total of flux oil equal to about  $\frac{1}{2}$  part flux oil to 1 part of fibre. A uniform dispersion of the pulverized asphalt and flux oil in the digested mass was then obtained and there was no difficulty with asphalt adhering to the screens while removing water by means of pressure. The sheets or pads thereby obtained contained about 60 to 70% of moisture and were passed through a drier at a temperature of about 250° F. and then repressed while hot. The resultant sheet or board was, on the average, 30% more waterproof than standard saturated asphalt roofing. The proportions of asphalt to fibre in the fibrous board were 1:1 by weight whereas the standard asphalt saturated sheet contains at least 1.6 of asphalt to 1 of fibre.

Alternately, it was found that if the mechanically broken up sugar cane or other fibrous material is mixed with the flux oil and allowed to stand for 1 to 2 weeks, very definite and material improvement is obtained not only in the dispersion of the flux oil and powdered asphalt and filler during the beating process but particularly in the water-proofing of the final product. It was found that the longer the mixture of mechanically disintegrated bagasse and flux oil is allowed to remain in the stock pile before cooking or digesting, the better is the subsequent dispersion in the beater and the more waterproof the finished product.

Lime may be used in the digestion and it is preferred in that it is relatively inexpensive and available in all localities.

Another desirable feature in using lime is that the lime soaps or any combination of lime with lignous material are invariably insoluble in water, whereas the products of reaction of lignous matter with caustic soda or soda sulfite or sulfate are all exceedingly water-soluble. When lime is used, it was found preferable that mechanically dis-

integrated bagasse and flux oil be premixed and allowed to soak for several days, and preferably for two weeks or longer.

It is not necessary that the asphalt be used in powdered form as it was found that high softening point low temperature susceptibility asphalt, for example having a softening point of about 140° to 240° F., may be used. As these particular high softening point-low susceptibility asphalts can not be pulverized in that they may be rubbery and tacky, they may be dispersed in stone dust or clay-water slurries to obtain an asphalt-clay-water paste wherein the asphalt is dispersed in extremely fine particles, in fact, considerably finer than current asphalt powders. The use of clay was found to be preferable over the use of stone dust as dry clay can be pulverized in a hammer mill and then plasticized with water at a lower cost than reducing lime stone or the like to a fineness below 200 mesh. Clay when properly plasticized makes a much finer filler than stone dust. By using clay or stone dust fillers with high softening point-low temperature susceptibility asphalt, a more pliable final product is obtained.

For example, mechanically disintegrated bagasse is mixed with flux oil and stored for one or two weeks and then digested with a lime solution of about 10% concentration for about 2 hours at about 100 lbs. per square inch steam pressure. This mass of digested disintegrated fibrous material and flux oil is next mixed with a clay-water-asphalt slurry, then dispersed as a pulp, and finally picked up by the continuous blanket of the wet machine. If a waterproof paper is being produced, the paper felt is removed from the blanket and passed through steam heated rolls for drying. If a waterproof board is being produced, the thick paper felt after being removed from the blanket is carried by a conveyor through a long hot air tunnel where it is dried.

Alternatively, asphalt cement, or a combination of asphalt cement with a heavy metal salt of an organic acid, such as aluminum naphthenate, copper naphthenate, etc., is dispersed in a mixture of clay and water to form an asphalt-clay-water paste. After this paste is formed, it can be reduced to a slurry of any desired consistency by incorporating additional water.

For example, mechanically disintegrated bagasse is mixed with flux oil and stored for one or two weeks or longer, and then digested with a lime solution of about 10% concentration for about 2 hours at about 100 pounds per square inch steam pressure. This mass of digested disintegrated fibrous material and flux oil is next mixed with a clay-water-asphalt slurry, (in which up to 75% of heavy metal salts of organic acids such as aluminum naphthenate, copper naphthenate, etc., may be incorporated in the bitumen), then dispersed as a pulp, and finally picked up by the continuous blanket of the wet machine. If a waterproof paper or paper felt is being produced, the thin felted layer is removed from the blanket and passed through steam heated rolls, or through a long hot air tunnel, for drying. If a waterproof paper board is being produced, the thick felted layer, after being removed from the blanket, is carried by a conveyor through a long hot air tunnel where it is dried.

It is sometimes desirable to introduce the waterproof material between layers of paper so that the waterproofing material would be contained in the inner portion of the sheet and

would not show on the outside layers. This may be readily done by forming one or more layers of paper felt introducing asphalt-clay-water suspension into one or more succeeding layers of paper felt, and finally covering with one or more layers of the paper felt, all of these operations being carried out as the layers of paper felt are being built up on the continuous blanket of the wet machine. This may be accomplished by either one or both of the following two methods:

1. In a paper machine consisting of several compartments, the clay-water-asphalt paste or slurry can be dispersed with the pulp in one or more of the central compartments, but not in the end compartments. In this way the blanket picks up a layer of paper pulp from the wet cylinder in the first one or more compartments, followed by a layer of paper pulp containing the clay-water-asphalt dispersion, from the wet cylinder in each of one or more of the central compartments, and finally picks up a layer of paper pulp alone from the wet cylinder in each of one or more compartments in the end of the machine. By this procedure, a waterproofed paper sheet or
- 25 paper board is obtained, which consists of central layers of pulp fibre impregnated with asphalt, contained within an envelope of outer layers of pulp fibre which do not contain asphalt.

2. This method is similar to (1) with the exception that in one or more of the central compartments of the wet machine, where the inner layers of the paper sheet or board are formed, the asphalt-clay-water slurry or paste is introduced into the pulp just as the fibre is being picked up by the wet cylinder, by spraying, etc.

In all cases, it should be clearly understood that the bituminous material used in the above processes for waterproofing and cementing purposes, may contain up to about 75% of metal salts of organic acids, such as aluminum naphthenate, copper naphthenate, etc. These compounds may be dissolved in the hard asphalt, in the flux oil, or both. They may also be added separately at some stage in the process, where they will combine with the bitumen, fibre, and mineral filler. These metal salts of organic acids modify the rigidity or pliability and other characteristics of the waterproofed paper sheet, paper felt, or paper board.

50 We claim:

1. A method of preparing a building composition which comprises breaking up a fibrous material into a state of fine subdivision, adding about  $\frac{1}{2}$  part of a flux oil to about 1 part of the divided fibrous material, adding an alkaline solution to the mixture of fibrous material and flux oil, digesting at 100 lbs. per square inch steam pressure for two hours the fibrous material, flux oil and alkaline solution to form a fibrous pulp, dispersing in the fibrous pulp an asphalt and flux oil, picking up the mixture of fibrous material, flux oil and asphalt in layers on a continuous blanket to form sheets, and submitting the said sheets of fibrous material, asphalt and flux oil to pressure and heat to remove water.

2. A method of preparing a building composition which comprises breaking up a fibrous material into a state of fine subdivision, adding about  $\frac{1}{2}$  part of a flux oil to about 1 part of the divided fibrous material, adding caustic soda to the fibrous material and flux oil, digesting at 100 lbs. per square inch steam pressure for two hours the fibrous material, flux oil and caustic soda to form a fibrous pulp, dispersing in the fibrous pulp an

asphalt and flux oil, picking up the mixture of the fibrous material, flux oil and asphalt in layers on a continuous blanket to form sheets, and submitting the said sheets of fibrous material, flux oil and asphalt to pressure and heat to remove water.

3. A method of preparing a building composition which comprises breaking up a fibrous material into a state of fine subdivision, adding about  $\frac{1}{2}$  part of a flux oil to about 1 part of the divided fibrous material, adding a solution of lime to the fibrous material, digesting at 100 lbs. per square inch steam pressure for two hours the fibrous material, flux oil and solution of lime to form a fibrous pulp, dispersing in the fibrous pulp an asphalt and flux oil, picking up the mixture of fibrous pulp, asphalt, flux oil and lime in layers on a continuous blanket to form sheets, and submitting the said sheets to pressure and heat to remove water.

4. A method of preparing a composition board which comprises mechanically subdividing a fibrous material, adding a flux oil to the finely divided fibrous material, allowing the mixture of finely divided fibrous material and flux oil to stand for at least seven days, adding a lime solution of about 10% concentration to the mixture of fibrous material and flux oil, digesting the mixture for about two hours at 100 pounds per square inch steam pressure, dispersing asphalt and flux oil in the mixture, picking up the mixture of fibrous material, flux oil, asphalt and lime in layers on a continuous blanket to form sheets, and submitting the said sheets to pressure and heat to obtain a composition board.

5. A method of preparing a composition board according to claim 4 in which asphalt is dispersed as a clay asphalt slurry containing copper naphthenate.

6. A method of preparing a composition board according to claim 4 in which the asphalt is dispersed as a clay-water-asphalt slurry.

7. A method of preparing a composition board according to claim 4 in which asphalt is dispersed as a clay-asphalt slurry containing a metal salt of naphthenic acid.

8. A method of preparing a composition of fibre board which comprises breaking up a fibrous material into a state of fine subdivision, impregnating about 1 part of the finely divided material with about  $\frac{1}{2}$  part of a flux oil, allowing the mixture to stand for at least seven days, adding lime to the mixture, digesting at 100 lbs. per square inch steam pressure for two hours the mix-

ture to form a fibrous pulp, dispersing asphalt with the fibrous pulp, picking up the mixture of fibrous pulp, flux oil, asphalt and lime in layers on a continuous blanket to form sheets, and submitting the said sheets to pressure and heat to form a board containing 1 part of asphalt, 1 part of the fibrous material.

9. A method of preparing a composition fibre board according to claim 8 in which the asphalt is dispersed as a stone dust asphalt water slurry.

10. A method of preparing a building composition which comprises breaking up a fibrous material into a state of fine subdivision, impregnating about 1 part of the finely divided fibrous material with about  $\frac{1}{2}$  part of a flux oil, allowing the mixture of fibrous material and flux oil to stand for at least several days, adding an alkaline solution to the mixture of finely divided fibrous material and flux oil, digesting at 100 lbs. per square inch steam pressure for two hours the mixture of finely divided fibrous material, alkaline solution and flux oil, dispersing asphalt and a metal salt of naphthenic acid in the fibrous material mixture, picking up the mixture of fibrous material, flux oil and asphalt in layers on a continuous blanket to form sheets, and submitting the sheets to pressure and heat to form a building composition containing 1 part by weight of asphalt to 1 part by weight of the fibrous material.

11. A method of preparing a building composition according to claim 10 in which the metal salt of naphthenic acid is aluminum naphthenate.

12. A method of preparing a building composition according to claim 10 in which the metal salt of naphthenic acid is copper naphthenate.

13. A method of preparing a building composition according to claim 10 in which 1 part of the fibrous material, 1 part of the asphalt and 1 part of a mineral filler are used.

CHARLES M. BASKIN,  
NORMAN W. MCLEOD.

#### REFERENCES CITED

The following references are of record in the file of this patent:

#### UNITED STATES PATENTS

| Number    | Name     | Date          |
|-----------|----------|---------------|
| 1,657,585 | Perry    | Jan. 31, 1928 |
| 1,754,343 | Waite    | Apr. 15, 1930 |
| 1,812,515 | Wagnon   | June 30, 1931 |
| 2,072,686 | Robinson | Mar. 2, 1937  |
| 2,132,607 | Davis    | Oct. 11, 1938 |
| 2,216,311 | Davis    | Oct. 1, 1940  |